

# UNITED STATES PATENT OFFICE.

CARL J. SCHNEIDER, OF NEW YORK, N. Y.

## FUEL-BRIQUET.

1,138,016.

Specification of Letters Patent.

Patented May 4, 1915.

No Drawing.

Application filed December 9, 1914. Serial No. 876,254.

*To all whom it may concern:*

Be it known that I, CARL J. SCHNEIDER, a citizen of the United States, and a resident of the city of New York, county and State 5 of New York, have invented new and useful Improvements in Fuel-Briquets, of which the following is a specification.

The purpose of the invention is to provide for the manufacture of briquets of coal 10 dust or waste, especially the dust or waste of anthracite coal, whereby the said coal dust or waste is given a marketable value, and is as well adapted for fuel as the lump coal, the product being similar in every respect to coal, burning with a lively fire, under complete combustion, and having high 15 caloric value.

In carrying out my invention, I first produce a mixture of molasses or of a similar 20 material with soap, while moderately heating said mixture say in a hot water bath, so as to incite the softening of the soap. I prefer to employ hard soda soap, which is advantageously reduced to small pieces or 25 shavings before being added to the molasses. After the soap has been sufficiently softened and a uniform mixture has been obtained, the latter is added to a suitable quantity of 30 coal dust or waste that has been reduced to a moderately fine powder. After these ingredients have been well intermingled in a suitable mixing machine, a solution of alum is added which has been previously dissolved 35 in about its own weight of boiling water, whereupon all of the above ingredients are thoroughly intermixed until a uniform mass is obtained in the form of a semi-dry powder. The latter is then molded into briquets 40 of convenient size by the aid of a power press, whereupon the briquets are dried in a current of warm dry air, to be then ready for shipment and use.

By the above described admixture of soap and alum to the molasses which constitutes 45 the binding agent proper, aluminum oleate will be formed owing to the action of the alum on the fatty or oleic acid of the soap, which aluminum oleate by being brought closely in contact with the small particles 50 of the coal and binder, acts as a waterproofing agent.

If the mixing of the above composition has been faithfully attended to, there is nothing more required; but I am well aware

that this work must of necessity be done 55 by unskilled labor which can not always be relied upon, and in order to make sure of a perfect product, I deem it advisable to treat the briquets further by passing the dried product first through a solution of soap and 60 then through one of alum, thereby forming a coating of aluminum oleate which adheres firmly to the briquets giving them an extra protection against absorption of 65 moisture. The strength of the solution of soap and alum may be regulated according to the thickness of the waterproof coating desired, the alum should, however, be in excess so as to completely neutralize the 70 soap.

In making up my improved composition for the molding of briquets, I use per each ton of coal dust, etc., about fifteen gallons of molasses, fifteen pounds of soap and twenty-five pounds of alum, but it is obvious 75 that such proportions may be varied without departing from the spirit of my invention.

From the above it is evident that the binding agent used, generates considerable heat of its own during combustion and therefore 80 does not act as an inert matter (such as cement, lime, plaster-of-Paris, etc.), it produces no unpleasant odor and burns without smoking. Briquets made as described, will hold in the fire so that they can be poked 85 like ordinary coal.

I claim:—

1. Process of making fuel briquets which consists in preparing a first mixture of molasses and soap, intermixing coal dust with 90 said first mixture to form a second mixture, adding a solution of alum to the second mixture, molding the mass thus obtained into briquets, and drying said briquets.

2. Process of making fuel briquets which 95 consists in preparing a first mixture of molasses and soap, intermixing coal dust with said first mixture to form a second mixture, adding a solution of alum to the second mixture, molding the mass thus obtained 100 into briquets, drying said briquets, and passing the dried briquets first through a solution of soap and then through a solution of alum.

3. Process of making fuel briquets which 105 consists in preparing a first mixture of fifteen gallons of molasses and fifteen pounds of soap, intermixing one ton of coal dust

with said first mixture to form a second mixture, adding a solution of twenty-five pounds of alum to the second mixture, molding the mass thus obtained into briquets,  
5 and drying said briquets.

4. A fuel briquet manufactured from a mixture of materials composed in about the

following proportions; one ton of coal dust, fifteen gallons of molasses, fifteen pounds of soap, and twenty-five pounds of alum.

CARL J. SCHNEIDER.

Witnesses:

ARTHUR E. ZUMPE,  
IDA O. KRUMM.